# EUROPEAN PATENT APPLICATION

(11) **EP 0 550 109 A1**
(43) Date of publication of application: **07.07.1993**
(21) Application number: 92204055.5
(22) Date of filing: 22.12.1992
(51) Int. Cl.: G03C 7/305

(54) **Photographic silver halide and process comprising a development facilitator**

(30) Priority: 30.12.1991 US 815727
(71) Applicant: EASTMAN KODAK COMPANY, Rochester, New York 14650-2201 (US)
(72) Inventor: Hill, Susan Dorothy, c/o Eastman Kodak Company, Rochester, New York 14650-2201 (US)
(74) Representative: Baron, Paul Alexander Clifford

(57) **Abstract**

A color photographic element comprising a support bearing at least one photographic silver halide emulsion layer containing at least one magenta image dye-forming coupler wherein the magenta image dye-forming coupler is at least one pyrazolo [3,2-c]-1,2,4-triazole, pyrazolo[1,5-b]-1,2,4-triazole or anilino-5-pyrazolone; and, the emulsion layer comprises a development facilitating concentration of a development facilitator coupler comprising a coupling-off group (A) that is represented by the formula -S-R⁸-R⁹ wherein R⁸ is alkylene containing 1 to 8 carbon atoms and R⁹ is a water solubilizing group, wherein the concentration of development facilitator coupler enables no bleach accelerator effect upon exposure and processing of the photographic element.

## Description

### Technical Field

This invention relates to a color photographic element comprising a development facilitating concentration of a development facilitator coupler.

Color photographic images in color photographic materials are commonly formed by a reaction between an oxidized silver halide developing agent and a dye-forming compound commonly called a coupler. This type of reaction has been well known in the photographic art. Such color photographic materials employed in the photographic art also contain light-sensitive silver halide emulsion layers.

### Assessment of the Art

One difficulty encountered with photographic silver halide materials is the need to reduce the concentration of silver which is required to provide a developed image. Attempts in the past to lower the concentration of photographic silver halide have not been entirely successful.

### Prior Art

Typical color photographic materials are described in, for example, U.S. Patent 4,980,267 and 4,982,996 and European Patent 193,389. However such patents do not disclose means for reducing silver halide concentrations in a color photographic silver halide material, particularly in the magenta layers of such a material.

### Disclosure of the Invention

The present invention provides for such a reduction in silver concentration by the use of a color photographic element comprising a support bearing at least one photographic silver halide emulsion layer containing at least one magenta image dye-forming coupler wherein the magenta image dye-forming coupler is at least one pyrazolo [3,2-c]-1,2,4-triazole, pyrazolo [1,5-b]-1,2,4-triazole or 1,2,4-anilino-5-pyrazolone; and, the emulsion layer comprises a development facilitator coupler in an amount sufficient to facilitate development, the development facilitator coupler comprising a coupling-off group (A) that is represented by the formula -S-R⁸-R⁹ wherein R⁸ is alkylene containing 1 to 8 carbon atoms and R₉ is a water solubilizing group, wherein the concentration of development facilitator coupler enables no bleach accelerator effect upon exposure and processing of the photographic element.

### Advantageous Effects of the Invention

The amount of the development facilitator coupler is a development facilitating concentration that enables a significant reduction in the concentration of photographic silver halide and or image dye forming coupler required to form a useful color image, especially a magenta image upon exposure and processing of the color photographic element. The concentration of photographic silver halide can be lowered by at least 5 wt% measured as silver ion with the concentration being lowered by a least 13 wt% to 25% and sometimes more.

Alternatively, the concentration of the image dye forming coupler can be reduced by at least 5 wt.% and typically by 23 to 37 wt.%. It will be appreciated both silver halide and image dye forming coupler can be reduced in combination to provide the most useful color image.

### A Detailed Account of at least one way of carrying out the Invention

The magenta image dye-forming coupler can be selected from a pyrazolo [3,2-C]-1,2,4-triazole, pyrazolo [1,5-b]-1,2,4-triazole, and anilino-5-pyrazolone.

A typical example of the pyrazolo [3,2-c]-1,2,4-triazole magenta image dye-forming coupler has the structure:
wherein:
R¹ and R² individually are substituents that do not adversely affect the coupling action of the coupler; X is hydrogen or a coupling-off group known in the photographic art.

According to formula(I), R¹ and R² individually represent hydrogen or a substituent. When R¹ is a substituent, it can be chosen from any of a number of well-known substituents for that position of a pyrazolo coupler, and is chosen so as to be compatible with the desired characteristics (e.g., activity, hue) of the coupler. Examples of substituents useful as R¹ include a substituted or unsubstituted alkyl group, (e.g., a methyl group, propyl group,) a t-butyl group, a trifluoromethyl group, a tridecyl group, a 3-(2,4-di-t-amylphenoxy) propyl group), a substituted or unsubstituted amyl group (e.g., a phenyl group, a 4-t-butylphenyl group, a 2,4,6,-trimethylphenyl group), a substituted or unsubstituted heterocyclic group (e.g., a 2-furyl group, a 2-thienyl group), a cyano group, a substituted or unsubstituted alkoxy group (e.g, a methoxy group, an ethoxy group), a substituted or unsubstituted aryloxy group (e.g., a phenoxy group, a 2-methylphenoxy group), a substituted or unsubstituted heterocyclic oxy group (e.g., a 2-benzimidazolyloxy group), a substituted or unsubstituted acyloxy group (e.g. an acetoxy group, a hexadecanoyloxy group), a substituted or unsubstituted caramoyloxy group (e.g., an N-phenylcarbamoyloxy group, an N-ethylcarbamoyloxy group), a substituted or unsubstituted silyoxy group (e.g., a trimethylsilyoxy group), a substituted or unsubstituted sulfonyloxy group (e.g., a dodecylsulfonyloxy group),a substituted or unsubstituted acylamino group (e.g., an acetamido group, a benzamido group), a substituted or unsubstituted anilino group (e.g., a phenylamino group, a 2-chloroanilino group), a substituted or unsubstituted ureido group (e.g., a phenylureido group, a methylureido group), a substituted or unsubstituted imido group (e.g., an N-succinimido group, a 3-benzylhydantoinyl group), a substituted or unsubstituted sulfamoylamino group (e.g., an N,N-dipropylsulfamoylamino group, an N-methyl-N-decylsulfamoylamino group), a substituted or unsubstituted carbamoylamino group (e.g., an N-butylcarbamoylamino group, an N,N-dimethylcarbamoylamino group), a substituted or unsubstituted alkylthio group (e.g., methylthio group, an octylthio group), a substituted or unsubstituted arylthio group (e.g., a phenylthio group, a 2-butoxy-5-t-octylphenylthio group), a substituted or unsubstituted heterocyclic thio group (e.g., a 2-benzothiazolyl group). a substituted or unsubstituted alkoxycarbonylamino group (e.g., a methoxycarboylamino group, a tetradecyloxycarbonylamino group), a substituted or unsubstituted aryloxycarbonylamino group (e.g., a phenoxycarbonylamino group, a 2,4-di-tert-butylphenoxycarbonylamino group) a substituted or unsubstituted sulfamido group (e.g., a methanesulfonamido group, a hexadecanesulfonamido group), a substituted or unsubstituted carbamoyl group (e.g., a N-ethylcarbamoyl group, an N,N-dibutylcarbamoyl group), a substituted or unsubstituted acyl (e.g., an acetyl group, a (2,4-di-tert-amylphenoxy)acetyl group), a substituted or unsubstituted sulfamoyl group (e.g., an N-ethylsulfamoyl group, an N,N-dipropylsulfamoyl group), a substituted or unsubstituted sulfonyl group (e.g., a methanesulfonyl group, an octanesulfonyl group, a sulfo group, a hydroxyl group, an amino group, and a carbonamido group, etc.) R¹ preferably represents an alkyl group, an aryl group, a carbonamido group, a sulfonamido group or sulfone group, a thio group, a sulfoxide group, a ureido group, or multicyclic group.

X represents a hydrogen atom or a group capable of being released by a coupling reaction with an oxidized aromatic primary amine developing agent (referred to herein as a coupling-off group). Coupling-off groups are known in the art and may include a group containing an aliphatic group, an aromatic group, a heterocyclic group, an aliphatic, aromatic, or heterocyclic carbonyl group that is bonded to the coupling active carbon via an oxygen atom, a nitrogen atom, a sulfur atom, or a carbon atom, a halogen atom, an aromatic azo group, and the like. The aliphatic, aromatic, or heterocyclic group contained in such coupling-off groups may have one or more substitutients, as described above for R¹.

Examples of coupling-off groups include a halogen atom (e.g., fluorine, chlorine, bromine), an alkoxy group (e.g., ethoxy, dodecyloxy, carboxypropyloxy), an aryloxy group (e.g., 4-chlorophenoxy group, a 4-methoxyphenoxy group), an acyloxy group (e.g., an acetoxy group, a tetradecanoyloxy group), an aliphatic or aromatic sulfonyloxy group (e.g., a methanesulfonyloxy group, a toluenesulfonyloxy group), an acylamino group (e.g., a dichloroacetylamino group, a trifluoroacetylamino group), an aliphatic or aromatic sulfonamido group (e.g., a methanesulfonamido group, a p-toluenesulfonamide group), an alkoxycabonyloxy group (e.g., an ethoxycarbonyloxy group, a benzyloxycarbonyloxy group), an aryloxycarbonyloxy group (e.g., a phenoxycarbonyloxy group), an aliphatic, aromatic or heterocyclic thio group (e.g., an ethylthio group, a phenylthio group), a carbamoylamino group (e.g., an N-methylcarbamoylamino group, an N-phenylcarbamoylamino group), a 5-membered or 6-membered nitrogen-containing heterocyclic group (e.g., an imidazolyl group, a pyrazolyl group), an imido group (e.g., a succinimido group, a hydantoinyl group), an aromatic azo group (e.g., a phenylazo group), and the like. Some of these groups may have substitutents selected from those described above for R¹.

Typical pyrazole [3,2-c]-1,2,4-triazole magenta image dye-forming couplers within the described structure are disclosed in, for example, U.S. Patents 4,777,121; 4,443,536; 5,019,489; European Patent 284,240; U.S. Patent 4,808,502; U.S. Patent 4,835,094; European Patent 285,274; and U.S. Patent 4,960,685.

Especially useful magenta image dye-forming couplers are:

Useful magenta image dye forming couplers include pyrazolotriazole couplers comprising pyrazolo-[1,5-b]-1,2,4-triazole couplers. Such couplers are represented by the formula:
wherein R¹, R² and X are defined above.

Typical pyrazolo [1,5-b]-1,2,4-triazole couplers are described in for example U.S Patents 4,540,654; 4,659,652; 4,774,172; 4,822,730; and 4,925,781; Japanese Published Patent Application No. 61-147254; European Patents 226,849;294,785; 119,860 and 234,428.

Examples of such couplers are:

Useful image dye forming couplers also comrise anilino-5-pyrazolone couplers. Such couplers include those represented by the formula:
wherein
R³ is a substitutent that does not adversely affect the coupling action of the coupler; typically an aryl group; preferably 2,4,6-trichlorophenyl;
R⁴ is an unsubstituted or substituted anilino group; and,
X is hydrogen or a coupling group known in the photographic art.

R³ is typically a substituted or unsubstituted aryl group (e.g., phenyl, 2-chlorophenyl, 4-chlorophenyl, 2,5-dichlorophenyl, 2,6-dichlorophenyl, 2,4,6-trichlorophenyl, 2-bromophenyl, 3,5-dibromophenyl, 2-cyanophenyl, 4-cyanophenyl, 3-nitrophenyl, 4-nitrophenyl, 4-methylphenyl, 2,6-dimethylphenyl, 2,6-diethylphenyl, 4-butylphenyl, 2-trifluoromethylphenyl, 2,6-dichloro-4-methoxycarbonylphenyl, 2,6-dichloro-4-tetradecyloxycarbonylphenyl, 2,6-dichloro-4-cyanophexyl, 2-ethoxyphenyl, 4-phenylphenyl, 4-phenoxyphenyl, 2-methyl-5-nitrophenyl, 2-chloro-5-cyano[henyl, 5-chloro-2-methylphenyl, 2,6-dichloro-4-methylphenyl, 2,4-dichloro-6-methoxycarbonylphenyl, 2,4-dichloro-6-methylphenyl, 2-chloro-4,6-dimethylphenyl, 2,6-dichloro-4-methoxyphenyl, 2,6-dichloro-4-nitrophenyl, 2,6-dichloro-4-acetamidophenyl, 2,6-dichloro-4-tetradecanamidophenyl, 2,4,6-trimethyl-3-nitrophenyl, 2,4,6-trimethyl-3-acetamidophenyl, etc.) or a heterocyclic group (e.g., 5- and 6-membered heterocyclic compounds such as 2-thiazolyl, 2-benthothiazolyl. 2-benzoxazolyl, 2-oxazolyl, 2-imidazolyl, 2-benzimidazolyl, etc.)

R⁴ is typically an unsubstituted or substituted anilino group represented by the formula:
wherein, R⁵ and R⁶ and R⁷ individually are hydrogen or a substituent that does not adversely affect the coupling action of the coupler, and at least one of R⁵, R⁶ and R⁷ is a ballast group known in the photographic art.

R⁵, R⁶ and R⁷ individually are, for example, hydrogen alkyl (e.g., methyl, t-butyl, octyl, and dodecyl), alkoxy (e.g., methoxy, ethoxy, octyloxy), alkylthio (e.g., methylthio, butylthio, dodecylthio), an amido group (e.g., acetamido, butyramido, methylsulfonamido, diacylamido, succinamido), a halogen atom (e.g., fluorine, chlorine, or bromine), a hydroxy group, a cyano group or a photographic ballast group known in the photographic art.

X is hydrogen or a coupling-off group as defined above.

Typical anilino-5-pyrazole couplers are described in, for example, U.S Patents 4,346,165; 3,907,571; 4,243,747; 2,343,703; 3,935,015; 4,351,897; 4,477,563; 4,853,319; 3,127,967; 3,519,429; 4,243,747; and 4,443,536; and, European Patent 226,664;

Examples of useful anilino-5-pyrazolone couplers are:

Combinations of magenta image dye-forming couplers are also useful.

As used herein development facilitating means the use of a compound that enables lowering of the silver halide concentration or coupler concentration or both and whose presence yields increased silver development. For example, the compound's presence can yield an increase in developed silver of at least 3% measured as developed silver in mg/m².

The development facilitating concentration is one which is effective in reducing the concentration of silver halide measured as silver ion and/or in reducing the concentration of magenta dye forming couplers which is required to provide a developed image.

More specifically the development facilitating concentration can range from 0.1 to 65 mg/m² of a development facilitator coupler, the coupler selected so as to avoid bleach acceleration.

Typically, the development-facilitating concentration can range from 0.25 to 33 mg/m². A development facilitator coupler, such as,
typically requires a development facilitating concentration within the range of 0.25 to 33 mg/m².

The development-facilitator coupler useful in the invention includes a coupling-off group (A) that is represented by the formula -S-R⁸-R9 wherein R⁸ is alkylene containing 1 to 8 carbon atoms, such as -CH₂-, -CH₂CH₂-,
or R9 is a water-solubilizing group, such as carboxyl.

A typical developing facilitating coupler is represented by the structure:
where COUP is a coupler moiety known in the photographic art such as a yellow, magenta or cyan dye forming coupler moiety, and the remainder of the molecule defined by S-R⁸-R⁹ is bonded to the coupling position of COUP, where R⁸ and R⁹ are as defined above.

A preferred color photographic element according to the invention comprises a preferred development facilitator coupler having the formula:
or

Typically the color photographic element comprises at least one red-sensitive photographic silver halide emulsion layer containing at least one cyan image dye-forming coupler, at least one green-sensitive photographic silver halide emulsion layer containing at least one magenta image dye-forming coupler and at least one blue-sensitive silver halide emulsion layer containing at least one yellow image dye-forming coupler and wherein the development facilitator coupler is in the green-sensitive silver halide emulsion layer.

In the following discussion of suitable materials for use in the emulsions and elements of this invention, reference will be made to Research Disclosure, December 1989, Item 308119, published by Kenneth Mason Publications, Ltd., Dudley Annex, 12a North Street, Emsworth, Hampshire P010 7DQ, ENGLAND, the disclosures of which are incorporated herein by reference. This publication will be identified hereafter by the term "Research Disclosure".

The silver halide emulsions employed in the elements of this invention can be either negative-working or positive-working. Suitable emulsions and their preparation are described in Research Disclosure Sections I and II and the publications cited therein. Suitable vehicles for the emulsion layers and other layers of elements of this invention are described in Research Disclosure Section IX and the publications cited therein.

In addition to the couplers generally described above, the elements of the invention can include additional couplers as described in Research Disclosure Section VII, paragraphs D, E, F and G and the publications cited therein. These couplers can be incorporated in the elements and emulsions as described in Research Disclosure Section VII, paragraph C and the publications cited therein.

The photographic elements of this invention or individual layers thereof, can contain brighteners (see Research Disclosure Section V), antifoggants and stabilizers (See Research Disclosure Section VI), antistain agents and image dye stabilizers (see Research Disclosure Section VII, paragraphs I and J), light absorbing and scattering materials (see Research Disclosure Section VIII), hardeners (see Research Disclosure Section IX), plasticizers and lubricants (See Research Disclosure Section XII), antistatic agents (see Research Disclosure Section XIII), matting agents (see Research Disclosure Section XVI) and development modifiers (see Research Disclosure Section XXI).

The photographic elements can be coated on a variety of supports as described in Research Disclosure Section XVII and the references described therein.

Photographic elements can be exposed to actinic radiation, typically in the visible region of the spectrum, to form a latent image as described in Research Disclosure Section XVIII and then processed to form a visible dye image as described in Research Disclosure Section XIX. Processing to form a visible dye image includes the step of contacting the element with a color developing agent to reduce developable silver halide and oxidize the color developing agent. Oxidized color developing agent in turn reacts with the coupler to yield a dye.

With negative working silver halide, the processing step described above gives a negative image. To obtain a positive (or reversal) image, this step can be preceded by development with a non-chromogenic developing agent to develop exposed silver halide, but not form dye, and then uniformly fogging the element to render unexposed silver halide developable. Alternatively, a direct positive emulsion can be employed to obtain a positive image.

Development is followed by the conventional steps of bleaching, fixing, or bleach-fixing, to remove silver and silver halide, washing and drying.
Coupler solvents useful in the present invention include:

### 2-Ethyl hexyl-p-hydroxybenzoate

### p- Dodecyl phenol

### 2,4-Di-t-pentyl phenol

The following examples further illustrate the invention:

### Example 1

A three color photographic film was prepared as follows using conventional surfactants, and antifoggants and the materials indicated. After providing a developable image and then processing in accordance with the Kodak C-41 process (British Journal of Photography, pp. 196-198(1988)) excellent results were obtained.

### Example 2

A three color photographic film was prepared as follows using conventional surfactants, and antifoggants and the materials indicated. After providing a developable image and then processing in accordance with the Kodak C-41 process (British Journal of Photography, pp. 196-198(1988)) excellent results were obtained.

### Couplers

1)
2)
3)
4)
5)
6)
7)
8)
9)
10)
11)
12)

### Dyes

(1)
(2)
(3)
(4) 4,8-bis-(SULFOMETHYLAMINO)-ANTHRARUFIN-2,6-DISULFONIC ACID, TETRASODIUM SALT
(5)
(6)
(7)
(8)

### Sensitizing Dyes

(1)
(2)
(3)
(4)
(5)

A photographic element in accordance with the invention was processed in Kodak C41 process at varying concentrations of development facilitator and was found to produce acceptable prints. The data from the processing is provided in Tables A and B.

Coupler solvent selection can influence stability of the photographic element when keeping. For example, improved stability can be observed when the coupler solvent (A) is used.

This invention has been described in detail with particular reference to preferred embodiments thereof. It will be understood that variations and modifications can be made within the spirit and scope of the invention.

## Claims

1. A color photographic element comprising a support bearing at least one photographic silver halide emulsion layer containing at least one magenta image dye-forming coupler wherein
a) the magenta image dye-forming coupler is at least one pyrazolo [3,2-c]-1,2,4-triazole, pyrazolo [1,5-b]-1,2,4-triazole or anilino-5-pyrazolone; and,
b) the emulsion layer comprises a development-facilitator coupler in an amount sufficient to facilitate development, the development facilitator coupler comprising a coupling-off group (A) that is represented by the formula - S-R⁸-R⁹ wherein R⁸ is alkylene containing 1 to 8 carbon atoms and R⁹ is a water solubilizing group, wherein the concentration of development facilitator coupler enables no bleach accelerator effect upon exposure and processing of the photographic element.

2. A color photographic element as in Claim 1 wherein the emulsion layer comprises a development facilitating concentration within the range of 0.1 to 65 mg/m² of the development facilitator coupler.

3. A color photographic element as in Claim 1 wherein the emulsion layer comprises a development facilitating concentration within the range of 0.25 to 32 mg/m² of the development facilitator coupler and the development facilitator coupler is a naphthol coupler.

4. A color photographic element as in any of claims 1-4 wherein the development facilitator coupler is a pyrazolo [3,2-c]-1,2,4-triazole coupler.

5. A color photographic element as in any of claims 1-4 wherein the development facilitator coupler is

6. A color photographic element as in any of claims 1-5 comprising at least one red-sensitive photographic silver halide emulsion layer containing at least one cyan image dye-forming coupler, at least one green-sensitive photographic silver halide emulsion layer containing at least one magenta image dye-forming coupler and at least one blue-sensitive photographic silver halide emulsion layer containing at least one yellow image dye-forming coupler and wherein the development facilitator coupler is in a green-sensitive photographic silver halide emulsion layer.

7. A color photographic element as in any of claims 1-6 comprising a support bearing, in sequence,
at least one red sensitive photographic silver halide emulsion layer comprising a cyan image dye-forming phenol coupler, a bleach accelerator releasing coupler and at least one development inhibitor releasing coupler;
at least one green sensitive photographic silver halide emulsion layer comprising at least one magenta image dye-forming pyrazolo [3,2-c]-1,2,4-triazole coupler, at least one development inhibitor releasing coupler, and a development facilitating concentration within the 0.25 to 33 mg/m² of the development facilitating coupler a yellow filter layer; and
at least one blue sensitive photographic silver halide emulsion layer comprising at least one pivalyl acetanilide yellow image dye-forming coupler, at least one alkoxyphenylacetanilide yellow image dye-forming coupler, at least one development inhibitor releasing coupler, and at least one development facilitating coupler.

8. A method of developing a color image in an exposed color photographic element as defined in any of claims 1-7 comprising developing the element with a color photographic silver halide developing agent.
